

Nov. 4, 1969

P. FABER

3,476,604

METHOD OF MAKING AN ELECTRODE GRID

Filed Sept. 15, 1967



Fig.1



Fig.2

2a Graphitized  
Carbonaceous  
Filament



Fig.3

Peter Faber  
INVENTOR

BY

Karl G. Ross  
Attorney

## 1

3,476,604

**METHOD OF MAKING AN ELECTRODE GRID**  
Peter Faber, Kahl am Main, Germany, assignor to  
Rheinisch-Westfälisches Elektrizitätswerk Aktien-  
gesellschaft, Essen, Germany, a corporation of  
Germany

Filed Sept. 15, 1967, Ser. No. 668,006

Claims priority, application Germany, Sept. 29, 1966,  
R 44,227

Int. Cl. H01m 35/04

U.S. Cl. 136—36

6 Claims

**ABSTRACT OF THE DISCLOSURE**

A grid for the electrodes of primary or secondary batteries, fuel cells and the like is produced by carbonizing a web of cellulose fibers which is thereafter heated to high temperatures, on the order of 2000° C., for at least superficial graphitization and is then metalized, preferably with a coating of nickel and boron, preparatory to having an active electrode material deposited thereon. The metalized graphite threads may be bonded together by sintering, preferably by the passage of a heating current therethrough.

My present invention relates to a grid for an electrode of an electrochemical cell, e.g. a fuel cell or a unit of a primary or secondary battery. Such grids serve the dual purpose of supporting the active electrode material and provide a low-resistance current path between the particles of such material.

An object of this invention is to provide a grid of this description which, taken by itself or when loaded with active electrode material, constitutes a porous body of large effective surface and low specific weight.

It is also an object of this invention to provide a simple and efficient method of producing such a body.

These objects are realized, in accordance with my present invention, by utilizing a web of carbonized and at least superficially graphitized filaments as a coherent skeleton on which a metallic coating is deposited to confer the necessary rigidity and conductivity upon the web. The metallic coating may be deposited from a suitable metalizing bath, with or without the application of a galvanizing voltage. Advantageously, this coating consists predominantly of nickel, the presence of a small proportion of boron (e.g. of about 5% by weight) in the composition being preferred. A coating of this description can be deposited, for example, from an aqueous solution of a nickel salt (e.g.  $\text{NiCl}_2$  or  $\text{NiNO}_3$ ) in the presence of a reducing boron compound (e.g. a borohydride such as  $\text{LiBH}_2$ ). Metalization by a simple redox process, without applied voltage, results in a substantially uniform distribution of the metallic deposit; the use of an electrolytic plating process, on the other hand, may lead to a denser deposit near the outer boundaries of the web which will usually not be objectionable.

Particularly with a nickel-containing coating, a thickness of about 5 to 10 $\mu$  for the metallic layer has been found very satisfactory.

The web of carbonaceous filaments to be metalized may be produced by charring a fabric or felt of cellulosic fibers and thereafter heating these fibers to a temperature on the order of 2000° C. for a time sufficient to result in at least superficial graphitization thereof. The charring step may

## 2

be carried out in an evacuated heating chamber or in a protective atmosphere.

Carbonaceous and graphitized filaments so obtained may have an overall thickness, together with their metallic coating, ranging between about 10 and 20 $\mu$ . The plate-shaped web itself may be originally up to 3.5 mm. thick, with a specific gravity of about 0.07 g./cm.<sup>3</sup> and an effective surface of up to 150 times its geometric area. The filaments may be sintered together by their coating, in order to strengthen the structure, by heating to a suitable temperature after metalization; this is advantageously done, e.g. in vacuo or in an atmosphere of a protective gas such as hydrogen, by the passage of a heating current through the web whose conductive filaments form a continuous current path. If desired, the porous body so obtained may be further compacted in a press before, during or after the sintering process; the resulting plate may have a thickness of 1–2 mm., though higher degrees of compaction (down to a fraction of a millimeter) are also possible.

The grid so produced may be loaded with active material, e.g. nickel hydroxide, cadmium hydroxide, silver oxide or zinc, by conventional processes such as pasting or vibration filling; this step may be omitted in the case of a fuel-cell electrode, e.g. for a cell of the air-zinc type.

The invention will be described in greater detail with reference to the accompanying drawing in which:

FIG. 1 shows a web of metalized carbonaceous filaments forming part of a grid according to the invention;

FIG. 2 is a fragmentary perspective view of one of the filaments of FIG. 1, drawn to a larger scale; and

FIG. 3 is a perspective view of a grid produced from the web of FIG. 1.

As shown in the drawing, a web 1 of metalized carbon filaments 3 is shaped into a rectangular plate having a terminal tab 4 attached thereto by spotwelding. As particularly illustrated in FIG. 2, each filament 3 consists of an inner core 2a of carbon coated with a metal layer 2b preferably having the aforescribed composition of 95% nickel and 5% boron.

A plate of this description is characterized by a surprising degree of elasticity, especially when compared with conventional electrodes made from sintered granular particles with or without imbedded reinforcements.

If a strip of felt or fabric of indefinite length is used to produce the web of FIG. 1, charring and metalization may be carried out in a continuous assembly-line-type process.

An electroless nickel-plating process of the type mentioned above has been disclosed in U.S. Patent No. 3,338,741.

I claim:

1. A method of making a grid for an electrode of an electrochemical cell, comprising the steps of carbonizing a web of cellulosic filaments, heating the carbonized web to a temperature on the order of 2000° C. for at least superficial graphitization, subsequently metalizing the filaments so obtained to provide them with a metallic coating and a low-resistance current path, and sintering said filaments together at their points of contact by passing an electric heating current through said filaments so coated.

2. A method as defined in claim 1 wherein said coating consists at least in major part of nickel.

3. A method as defined in claim 2 wherein said coating is a composition of nickel and boron, the latter being present in a proportion of substantially 5% by weight.

4. A method as defined in claim 2 wherein said coating has a thickness ranging substantially between 5 and 10 $\mu$ .

5. A method as defined in claim 4 wherein said fila-

ments have an overall thickness ranging between substantially 10 and 20 $\mu$ .

6. A method as defined in claim 1, further comprising the step of compacting said web of filaments.

|           |         |                 |       |         |
|-----------|---------|-----------------|-------|---------|
| 3,192,071 | 6/1965  | Vinal           | ----- | 136—121 |
| 3,222,224 | 12/1965 | Williams et al. |       |         |
| 3,343,990 | 9/1967  | Giddy           | ----- | 136—36  |

## References Cited

## FOREIGN PATENTS

|           |        |         |
|-----------|--------|---------|
| 1,155,740 | 5/1958 | France. |
|-----------|--------|---------|

## UNITED STATES PATENTS

|           |         |                |       |         |
|-----------|---------|----------------|-------|---------|
| 536,996   | 4/1895  | Barnett        | ----- | 136—121 |
| 2,658,099 | 11/1953 | Basset         | ----- | 136—121 |
| 2,865,973 | 12/1958 | Hartman et al. | ----- | 136—64  |
| 3,071,637 | 1/1963  | Horn et al.    | ----- | 136—36  |
| 3,183,123 | 5/1965  | Haworth.       |       |         |

|                                      |
|--------------------------------------|
| WINSTON A. DOUGLAS, Primary Examiner |
|--------------------------------------|

|                                    |
|------------------------------------|
| C. F. LEFEVOUR, Assistant Examiner |
|------------------------------------|

|               |
|---------------|
| U.S. Cl. X.R. |
|---------------|

|                      |
|----------------------|
| 75—201, 212; 136—122 |
|----------------------|